

Patented Mar. 22, 1927.

1,622,099

# UNITED STATES PATENT OFFICE.

WILLIAM FELDENHEIMER, OF LONDON, ENGLAND.

## TREATMENT OF EARTHY MINERALS.

No Drawing.

Application filed October 30, 1925. Serial No. 65,892.

My invention relates to the treatment of clays or like earthy minerals for their purification and improvement of their color. In my copending application, Serial No. 33,051, filed May 26, 1925 I have described the treatment of such minerals with an acid salt of sulphurous acid in the presence of a metal such as zinc. I have now discovered that instead of bringing the earthy mineral in contact with acid salt of sulphurous acid in the actual presence of metallic zinc or other metal, I can prepare a bleaching liquid by digesting the zinc or other metal in a salt of sulphurous acid and can thereafter treat the earthy mineral, such as clay slip, with this liquor and obtain a result similar to that of the process of my copending application above referred to without the presence of the metal in the treatment bath. The zinc or other metal should be in excess in this step.

As stated in the specification of my application Serial No. 33,051, the use of an acid such as sulphurous acid, has certain disadvantages in commercial use. The acid is difficult to handle and liable to attack the plant apparatus; and is also readily oxidized to produce the more corrosive sulphuric acid. The action of sulphurous acid upon metal tends to be localized by reason of the use of a gas and in bulk operation it is difficult to insure uniform treatment of the mineral. In accordance with the present invention, the earthy mineral such as clay which is to be improved in color, is brought into contact with a liquor which has been formed by digesting metal such as zinc in a salt of sulphurous acid. The salt of sulphurous acid is preferably sodium bisulphite or sodium metabisulphite, and the metal used is preferably a metal such as zinc which does not form oxidized colored salts.

A difficulty in the bleaching of clay is that the clay after having been treated with bleaching agents becomes recolored upon drying, and if a metal, such as iron, which yields colored oxidized salts to be employed in the reaction, the object of the bleaching process may be partly or wholly defeated, but if used in every dilute concentration such metal may as a catalyst hasten the bleaching.

It is of advantage at times, in order to accelerate the reaction, to add to a trace of a mineral acid to the reaction mixture, preferably an acid which yields the less readily oxidized salts of iron, for example, hydrochloric acid. Bleaching will proceed, how-

ever, without the presence of the acid. Sodium sulphite may be used with zinc for example, provided a small quantity of acid such as hydrochloric acid is present. Since the earthy minerals and clays differ in character, the treatment must be varied according to the particular earthy mineral being treated.

In carrying the invention into effect, care should be observed to maintain efficient agitation of the mineral suspension throughout the operation in order to insure as complete and uniform an action as possible upon the mineral.

I have found that the liquor formed by digesting zinc in sodium bisulphite or sodium metabisulphite will bleach certain clays which are not bleached by zinc and sulphurous acid.

The liquor which I employ probably contains sodium hydrosulphite, sodium sulphite and sulphite of zinc or other metal employed and the present process is an improvement over that of my copending case, in that no provision need be made for the presence of a metal such as zinc, in the bath where the clay or earthy mineral is treated.

With the use of my invention the bleaching action is more efficient and rapid and extends throughout the bath instead of being localized.

Acidity, if used, is only of advantage in rapidly liberating the acids and gases which carry out the bleaching action.

The coloring matter may be decanted off with the excess water; and this should be done if the fluid is exposed to air and sunlight as substances in the upper water layer will usually become yellowish or brownish on such exposure.

Changes may be made in the particular salt of sulphurous acid and in the metal employed provided the metal reduces  $SO_2$ .

I claim:

1. In the process for improving the color of earthy minerals, the step comprising ring-  
ing an aqueous suspension of the sub-divided mineral into contact with a salt of sulphurous acid containing a salt of a metal which reduces sulphurous acid and does not form colored oxidized salts.

2. In the process of improving the color of earthy minerals, the step comprising bring-  
ing into contact with an aqueous suspension of the sub-divided mineral a salt of sulphurous acid containing a salt of zinc.

3. In the process for improving the color of clay, the step consisting in bringing in contact with the clay in suspension in water a sulphite salt of sodium in the presence of a salt of a metal which reduces sulphurous acid and does not form colored oxidized salts.

4. In the process for improving the color of clay, the step consisting in bringing in contact with the clay in suspension in water sodium metabisulphite in the presence of a salt of zinc.

5. In the process for improving the color of clay, the step consisting in bringing in

contact with the clay in suspension in water 15 a sulphite salt of sodium in the presence of acid and a salt of a metal which reduces sulphurous acid and does not form colored oxidized salts.

6. In the process for improving the color 20 of clay, the step consisting in bringing into contact with the clay in suspension in water a salt of hydrosulphurous acid and a salt of a metal which reduces sulphurous acid and does not form colored oxidized salts. 25

In testimony whereof I have hereunto set my hand.

WILLIAM FELDENHEIMER.